

Sept. 1, 1970

AKIRA SASANO ET AL

3,526,543

PHOTOCONDUCTIVE FILM

Filed Jan. 31, 1967



INVENTORS

AKIRA SASANO  
MITSURU OIKAWA

BY

*Paul M. Craig, Jr.*

ATTORNEY

**1****3,526,543****PHOTOCONDUCTIVE FILM**

Akira Sasano, Kokubunji-shi, and Mitsuhiro Oikawa, Tokyo, Japan, assignors to Hitachi, Ltd., Tokyo, Japan, a Japanese corporation

Filed Jan. 31, 1967, Ser. No. 612,866

Claims priority, application Japan, Feb. 28, 1966,  
41/11,678

Int. Cl. B44d 1/18

U.S. Cl. 117—217

7 Claims

**ABSTRACT OF THE DISCLOSURE**

A photoconductive film to be used as a target of a vidicon and the like, said film being formed by laminating a film layer of metal and a photoconductive layer upon a conductive transparent layer and characterized in that the photoelectric current is increased by reducing the dark current.

This invention relates to an improvement in a photoconductive film to be used as a target of a vidicon and the like, and it is an object of the invention to provide a sensitive photoconductive film wherein the photoelectric current is increased by reducing the dark current.

Other objects, features and advantages of the invention will become apparent from the following detailed description of the invention when taken in conjunction with the accompanying drawings, in which:

The drawing is a sectional diagram of photoconductive film embodying the present invention.

A conventional photoconductive film used as a target of a visual vidicon has been formed by laminating a conductive transparent layer and a photoconductive layer on a glass substrate which constitutes a vidicon tube. In this apparatus, the variation in the electrical conductivity of the photoconductive layer caused by the incident light is converted to the variation in the current of the radiating electron beam, and said variation is detected as an output current by the conductive transparent layer which works as a signal electrode. Among the photoconductive films of this kind, a film which employs a NESA film ( $\text{SnO}_2$ , trademark) as the conductive transparent layer 2 and  $\text{Sb}_2\text{S}_3$  film as the photoconductive layer has a transparent signal electrode and enjoys a high electrical conductivity. Therefore, this photoconductive film works rather well. However, since the dark current is large in this device, it is impossible to increase the photoelectric current.

In order to improve said defect, an attempt has been made to employ a semitransparent evaporated metal layer as the signal electrode, but since the transverse electrical conductivity is required for the signal electrode, the layer must be thick. This, in turn, lowers the transparency of the layer and thus it has been difficult to put said layer to practical use.

The present invention is intended to obviate the deficiencies described above.

The present invention consists of a photoconductive film formed by laminating a film layer of metal and a photoconductive layer on a conductive transparent layer.

The drawing shows an example of the photoconductive film according to the invention, wherein reference numeral 1 designates a glass substrate, 2 a conductive transparent layer, 3 a film layer and 4 a photoconductive layer. Good results were obtained with this device when the conductive transparent layer 2, the film layer 3, the photoconductive layer 4 were made to be 300–600 Å., 10–100 Å. and 3–5 μ in thickness, respectively.

The existence of said film layer 3 changes the form of the energy bands of the photoconductive body by the contact thereof with the photoconductive layer and ac-

**2**

cordingly, by suitably selecting the metal to be used for the film layer, the contactness with the photoconductive layer can be freely changed. Thus, the electrical resistance of the photoconductive layer can be increased and thereby the characteristics of the photoconductive layer can be improved.

In a photoconductive film formed in this way, both the film layer 3 and the conductive transparent layer 2 work as a signal electrode and, in addition, the conductive transparent layer 2 has a high electrical conductivity. Therefore, the film layer 3 may not have a high electrical conductivity and so a thin evaporated film or the like can be used as said film layer. Thus, the reduction of the transparency against the incident light can be minimized.

The metals most used for the film layer are Ag, Al and Cu and they are particularly suitable when the photoconductive layer is formed of  $\text{As}_2\text{Se}_3$ ,  $\text{As}_2\text{Se}_2\text{S}$ ,  $\text{As}_2\text{Se}_2\text{S}_2$ ,  $\text{As}_2\text{S}_3$ , or Se.

Now, the embodiments of the invention will be described.

**EMBODIMENT 1**

As the film layer, Ag is evaporated on a NESA film adhered to a glass substrate. Upon said film layer is evaporated  $\text{As}_2\text{Se}_3$  to form a photoconductive layer and thus a photoconductive target is provided. When this target is used with a target voltage of 60 v., the dark current is 0.005 μa. and the photoelectric current is 0.2 μa. with an illumination of 2.5 lux. On the other hand, in a conventional target consisting of a NESA film and an evaporated  $\text{As}_2\text{Se}_3$  film, the dark current is 0.03 μa. and the photocurrent is 0.1 μa. with an illumination of 10 lux when said conventional target is used with a target voltage of 5 v. Thus, the reduction of a dark current and the increase of a photocurrent are achieved.

**EMBODIMENT 2**

As the film layer, Al is evaporated on a NESA film adhered to a glass substrate. On said film layer is evaporated  $\text{As}_2\text{Se}_3$  to form a photoconductive layer and thus a photoconductive target is provided. When this target is used with a target voltage of 20 v., the dark current is 0.004 μa. and the photoelectric current is 0.3 μa. with an illumination of 2.5 lux. Also in this case, comparison with the known target as described in Embodiment 1 shows that a good result is obtained with this novel target.

**EMBODIMENT 3**

As the film layer, Al is evaporated on a NESA film adhered to a glass substrate. On said film layer is evaporated  $\text{As}_2\text{Se}_2\text{S}$  to form a photoconductive layer and thus a photoconductive target is provided. When this target is used with a target voltage of 50 v., the dark current is 0.002 μa. and the photocurrent is 0.1 μa. with an illumination of 2.5 lux. On the other hand, when a conventional target consisting of a NESA film and an evaporated  $\text{As}_2\text{Se}_2\text{S}$  film is used with a target voltage of 10 v., the dark current is 0.012 μa. and the photoelectric current is 0.08 μa. with an illumination of 10 lux. Thus, evidently the reduction of a dark current and the increase of a photocurrent are achieved.

**EMBODIMENT 4**

As the film layer, Al is evaporated on a NESA film adhered to a glass substrate. On said film layer is evaporated  $\text{As}_2\text{Se}_2\text{S}_2$  to form a photoconductive layer and thus a photoconductive target is provided. When this target is used with a target voltage of 50 v., the dark current is 0.002 μa. and the photoelectric current is 0.05 μa. with an illumination of 2.5 lux. On the other hand, when a conventional target consisting of a NESA film and an evaporated  $\text{As}_2\text{Se}_2\text{S}_2$  film is used with a target voltage

of 30 v., the dark current is 0.01  $\mu$ a. and the photocurrent is 0.05  $\mu$ a. with an illumination of 10 lux. Thus, the reduction of a dark current and the increase of a photocurrent are achieved.

It is to be noted that the increase in dark current due to the passage of time, as seen in a conventional target consisting of a NESA film and an evaporated film of  $As_2Se_3$ ,  $As_2Se_2S$ ,  $As_2SeS_2$  or the like, is not found in the photoconductive target according to Embodiments 1 to 4. This fact is also preferable for increasing the sensitivity of a photoconductive layer. Further, though the embodiments using Al or Ag for the film layer are described hereinabove, other kinds of metal like Cu can also be used to obtain the same effect.

As is fully described hereinabove, the photoconductive film according to the invention can reduce the dark current present at a conventional photoconductive target consisting of a conductive transparent layer and photoconductive layer. Accordingly, it has become possible to increase a target voltage and hence to increase the photoelectric current. Also, the increase with time of the dark current can be prevented.

Further, since both the conductive transparent layer and the film layer work as a signal electrode in the photoconductive film according to the invention, the contactness with the photoconductive layer can be adjusted by suitably selecting the film layer. The invention can equally be applied to the case where  $As_2S_3$ , Se or the like is used for the photoconductive layer. Thus, the present invention makes it possible to fabricate a photoconductive film having good characteristics unattainable by a conventional film consisting of a conductive transparent layer and a photoconductive layer, and hence it has become possible to provide a highly efficient vidicon. Therefore, the present invention has a wide range of industrial applications.

What is claimed is:

1. A photoconductive film consisting essentially of a substrate, a conductive transparent layer of a material which is more transparent than a correspondingly conductive semitransparent metal layer formed on said substrate, a metal film selected from the group consisting of Al, Ag, and Cu films on said conductive transparent layer, and a photoconductive layer consisting of a mate-

rial selected from the group consisting of  $As_2Se_3$ ,  $As_2Se_2S$ ,  $As_2SeS_2$  and  $As_2S_3$ , said metal film providing a layer of high electric resistance as a result of the contact thereof with said photoconductive layer.

2. A photoconductive film as defined in claim 1, wherein in said metal film comprises Al and said photoconductive layer is  $As_2Se_3$ .

3. A photoconductive film as defined in claim 1, wherein in said metal film comprises Ag.

4. A photoconductive film as defined in claim 1, wherein in said metal film comprises Cu.

5. A photoconductive film as defined in claim 1, wherein in the thickness of (a) the conductive transparent layer is about 300-600 angstroms, (b) the metal film is about 10-100 angstroms and (c) the photoconductive layer is about 3-5  $\mu$ .

6. A photoconductive film consisting essentially of a substrate, a conductive transparent layer comprising  $SnO_2$  formed on said substrate, a metal film selected from the group consisting of aluminum, silver and copper formed on said conductive transparent layer, and a photoconductive layer consisting of a material selected from the group consisting of  $As_2Se_3$ ,  $As_2Se_2S$ ,  $As_2SeS_2$  and  $As_2S_3$ , said metal film providing a layer of high electric resistance as a result of the contact thereof with said photoconductive layer.

7. A photoconductive film as defined in claim 6, wherein in the thickness of (a) the conductive transparent layer is about 300-600 angstroms, (b) the metal film is about 10-100 angstroms and (c) the photoconductive layer is about 3-5  $\mu$ .

#### References Cited

##### UNITED STATES PATENTS

|    |           |         |                    |         |
|----|-----------|---------|--------------------|---------|
| 35 | 2,822,300 | 2/1958  | Mayer et al. ----- | 117-201 |
|    | 2,833,675 | 5/1958  | Weimer -----       | 117-201 |
|    | 2,844,543 | 7/1958  | Fotland -----      | 117-201 |
|    | 3,350,595 | 10/1967 | Kramer -----       | 117-217 |

ALFRED L. LEAVITT, Primary Examiner

C. K. WEIFFENBACH, Assistant Examiner

U.S. CL. X.R.

117-227; 313-94